



US005336557A

# United States Patent [19]

Takamatsu et al.

[11] Patent Number: 5,336,557

[45] Date of Patent: Aug. 9, 1994

[54] CARBON FIBER FELTING MATERIAL AND  
PROCESS FOR PRODUCING THE SAME

[75] Inventors: Akio Takamatsu; Yoshiyuki  
Nishimura, both of Kamisu, Japan

[73] Assignee: Petoca Ltd., Tokyo, Japan

[21] Appl. No.: 748,726

[22] Filed: Aug. 22, 1991

## [30] Foreign Application Priority Data

Aug. 23, 1990 [JP] Japan ..... 2-220061

[51] Int. Cl.<sup>5</sup> ..... B32B 5/06; B32B 11/10;  
B32B 31/16; B32B 31/26; D01F 9/145

[52] U.S. Cl. ..... 428/300; 52/782;  
156/62.4; 156/62.8; 156/148; 156/300;  
423/447.1; 423/447.2; 428/367; 428/408;  
428/920

[58] Field of Search ..... 428/367, 408, 920, 300;  
156/62.4, 62.8, 148, 300; 423/447.1, 447.2

## [56] References Cited

### U.S. PATENT DOCUMENTS

4,014,725 3/1977 Schulz ..... 156/148  
4,350,672 9/1982 Layden, Jr. et al. ..... 423/445  
4,628,001 12/1986 Sasaki et al. ..... 428/367  
4,776,994 10/1988 Nelson et al. ..... 264/29.2

4,849,200 7/1989 Uemura et al. ..... 423/447.4  
4,868,037 9/1989 McCullough et al. ..... 428/367  
4,898,783 2/1990 McCullough et al. ..... 428/408  
4,977,023 12/1990 Krupp et al. ..... 428/408  
5,034,267 7/1991 McCullough et al. ..... 428/408  
5,035,942 7/1991 Nagata et al. ..... 428/408  
5,047,292 9/1991 Salanobu et al. ..... 428/367  
5,057,341 10/1991 Ogiso et al. ..... 428/408  
5,068,061 11/1991 Knobel et al. ..... 428/408

## FOREIGN PATENT DOCUMENTS

0386633 9/1990 European Pat. Off. .

Primary Examiner—James C. Cannon  
Attorney, Agent, or Firm—Armstrong, Westerman  
Hattori, McLeland & Naughton

## [57] ABSTRACT

The disclosed carbon fiber felting material has a bulk density of 0.01 to 0.5 g/cm<sup>3</sup> and a thermal conductivity of at most 1.0 kcal/m·hr·°C. in the thickness-wise direction thereof at 2,200° C. The carbon fiber felting material is formed through physical and/or chemical interfiber entanglement. The carbon fiber felting material is very stable in an inert atmosphere, and excellent in heat insulating properties in a high-temperature range and against radiant heat transfer in particular.

3 Claims, No Drawings

## CARBON FIBER FELTING MATERIAL AND PROCESS FOR PRODUCING THE SAME

### BACKGROUND OF THE INVENTION

#### 1. Field of the Invention

The present invention relates to a heat-insulating, carbon fiber felting material excellent in heat insulating properties, particularly in a high temperature range.

More particularly, the present invention relates to a carbon fiber felting material which exhibits excellent heat resistance and morphological stability within the temperature range of 500° to 2,800° C. as well as excellent heat insulating properties against radiant heat transfer in particular.

Still more particularly, the present invention relates to a carbon fiber felting material so excellent in heat insulating properties within the high temperature range that the felting material can be used for heat insulation of high temperature furnaces and the like which are used in fusion of glass, firing of pottery, smelting of metals, sintering of ceramics, or heat treatment of carbonaceous materials.

The present invention further relates to a carbon fiber felting material so excellent in stability against thermal radiation that the felting material can be used as a heat insulating material with excellent performance in nuclear furnaces and nuclear power generating installations.

#### 2. Related Art

Porous ceramic materials have heretofore been mostly used as heat insulating materials serviceable within a high temperature range. These heat-insulating ceramic materials have an excellent high-temperature stability. In order to lower the thermal conductivity, however, they are required to have a considerable porosity.

The pores of the porous ceramic materials are not of completely closed-cell type, but usually is considerably restrictive on gaseous flow therethrough. This is so, from the viewpoint of strength, because those pores are formed in such a way as to communicate with the outsides of the porous ceramic materials only through considerably small passages. This will be understandable if consideration is given to the fact that any shaped ceramic article is decreased in strength in the case where it includes so large defects around the peripheries of its pores as to allow a gas to easily flow therethrough.

Because of such morphological characteristics, the conventional heat-insulating ceramic materials are generally so weak against rapid cooling as well as rapid heating that they may involve a problem of frequent structural collapse beginning with the surfaces thereof upon changes of the temperature, which is called "spalling." In order to provide a heat-insulating ceramic material hardly subject to spalling, it is generally necessary to select a ceramic material low in porosity and hence poor in heat insulating properties, which must, therefore, be used in large amount.

As a solution to the foregoing problems, fibrous ceramic materials have heretofore been widely used as heat insulating materials. The fibrous ceramic materials exhibit an excellent heat insulating effect. However, they are generally expensive due to a difficulty encountered in production thereof. This is one reason for the high price of a high-temperature furnace.

On the other hand, the predominant mode of heat transfer shifts to radiant heat transfer with relatively

decreasing contribution of convective as well as conductive heat transfer when the temperature reaches the high-temperature range of at least 500° C. This presents a problem that, when the performance of a heat insulating material is considered in association with an aspect of its heat insulation mechanism, the heat insulating material effective in the low-temperature range of at most 200° C. does not necessarily exhibit good performance in the high-temperature range.

Particularly, heat-insulating fibrous ceramic materials exhibit an excellent heat insulating effect in the low-temperature region, but are so poor in capability of radiation absorption and scattering as to provide an insufficient heat insulating effect against radiant heat transfer in the high-temperature range, because of their generally high transparency and very high surface smoothness characteristic of such fibers.

On the other hand, either carbonaceous or graphitic materials, e.g., mesophase pitch type materials in particular have heretofore attracted attention of little significance as heat insulating materials because they are generally high in thermal conductivity to allow for large conductive heat transfer therethrough.

Since these materials are high in absorbance for radiations ranging from ultraviolet radiation to infrared radiation within a wide wave range and endowed with high morphological stability at high temperatures, however, it has been believed that they could probably be used as heat insulating materials if they were provided with a morphology highly capable of radiation scattering.

An object of the present invention is to provide a heat insulating material which can solve not only the problem that the conventional heat insulating materials for use in the high-temperature range are weak against rapid temperature changes and generally insufficient in the heat insulating effect against radiant heat transfer, but also the problem that the heat-insulating, fibrous ceramic materials are generally expensive and insufficient in the heat insulating effect against radiant heat transfer.

### SUMMARY OF THE INVENTION

As a result of extensive investigations with a view to solving the above-mentioned problems, the authors of the present invention have found out that a felting material produced through such entanglement of a thin carbon fiber material as to take the form of a high bulk density felt is very useful as a heat insulating material in the high-temperature range since it is very low in thermal conductivity especially in the thickness-wise direction of the felt. The present invention has been completed based on this finding.

More specifically, in accordance with one aspect of the present invention, there is provided a carbon fiber felting material excellent in heat insulating properties in the high-temperature range: which is substantially in the form of a felt formed through interfiber entanglement and having a bulk density of 0.01 to 0.5 g/cm<sup>3</sup> and a thermal conductivity of at most 1.0 kcal/m·hr·°C. in the thickness-wise direction thereof at a temperature of 2,200° C.

The carbon fiber used in the carbon fiber felting material of the present invention preferably has an average filament diameter of 1 to 9  $\mu\text{m}$ .

The carbon fiber is preferably of a pitch type, more preferably of a mesophase pitch type having a moisture

absorption of at most 2 wt. % in an atmosphere having a temperature of 20° C. and a relative humidity of 65%.

In accordance with another aspect of the present invention, there is provided a process for producing a carbon fiber felting material excellent in heat insulating properties: comprising the step (1) of spinning a starting pitch material by a melt blow method and collecting the spun fiber into the form of a sheet, the step (2) of subjecting the fiber sheet to infusibilization and subsequent slight carbonization treatments, and the step (3) of piling up a desired number of the resultant carbon fiber sheets and subsequently entangling the carbon fiber sheets with each other, followed by carbonization of the resultant mat if desired.

#### DETAILED DESCRIPTION

The present invention will now be described in more detail.

#### CARBON FIBER

A carbon fiber preferably having an average filament diameter of 1 to 9  $\mu\text{m}$  is used in the carbon fiber felting material of the present invention.

Additionally stated, the average filament diameter of the carbon fiber subjected to the slight carbonization treatment but before being subjected to the entanglement treatment such as needle punching is slightly larger (by about 10%) than the average filament diameter of the final carbon fiber heat-treated at a high temperature.

The average filament diameter is expressed by an average value of the diameters of, for example, 100 randomly sampled filaments which are measured through an optical microscope or an electron microscope.

The thermal conductivity of a heat-insulating material as used in the high-temperature range, in the thickness-wise direction thereof at a temperature of 2,200° C., is desired to be at most 1.0 kcal/m·hr·°C., preferably at most 0.7 kcal/m·hr·°C. When the average filament diameter exceeds 9  $\mu\text{m}$ , a difficulty is encountered in holding down the thermal conductivity, as mentioned above, of the carbon fiber felting material at or below 1.0 kcal/m·hr·°C. When the average filament diameter is smaller than 1  $\mu\text{m}$ , various troubles, including incorporation of odd-shaped particles other than fibrous materials and breakage of filaments, are unfavorably liable to occur in the step of fiber spinning from pitch in particular.

The use of the carbon fiber having a small filament diameter as the fiber to constitute the felting material greatly enhances the heat insulating effect against radiant heat transfer.

When consideration is given, for example, to spinability into such a morphology as to provide a high heat insulating effect, the carbon fiber is preferably of a pitch type, such as a petroleum pitch type or a coal pitch type, especially preferably of a mesophase pitch type. In addition, however, carbon fibers respectively produced from polyacrylonitrile, rayon, and novolak resin as the starting materials can be used in the present invention.

The moisture absorption of the carbon fiber is desired to be as low as possible. The moisture absorption particularly in an atmosphere having a temperature of 20° C. and a relative humidity of 65% is preferably at most 2%, more preferably at most 0.1%.

Among various pitch type carbon fibers, a mesophase pitch type carbon fiber is comparatively low in moisture

absorption and hence provides favorable properties for the carbon fiber felting material of the present invention produced therefrom.

The above-mentioned value of moisture absorption is a proportion of the weight of absorbed water relative to the weight of the felting material.

When a carbon fiber felting material having a high moisture absorption is used as a heat insulating material, evaporation of absorbed moisture occurs during the course of heat-up thereof from room temperature to unfavorably lower the heat insulating effect of the heat insulating material. In addition, such a carbon fiber felting material gives out steam into the atmosphere surrounding the carbon fiber to cause deterioration of the carbon fiber at high temperatures.

#### ENTANGLEMENT

The carbon fiber felting material of the present invention substantially keeps the morphology thereof thanks to the interfiber entanglement thereof.

The term "entanglement" used herein is not restricted to "physical entanglement" in a narrow sense, but is intended to encompass any chemical and/or physical interfiber entanglement in so far as a carbon fiber aggregate randomly gathered in a spread state can be formed thereby into a felty material.

##### (A) Physical Entanglement

General physical entanglement treatments employable in the present invention include entanglement with turbulent gaseous flow, entanglement with penetrating columnar liquid flow, and entanglement by needle punching, etc. Interfiber entanglement by needle punching is preferable from the viewpoint of avoiding putting fiber orientation in the thickness-wise direction of the felting material into disarray.

##### (B) Entanglement with Binder

Interfiber application of a binder is effective as chemical entanglement to keep the carbon fiber in the form of a felting material. Such binder application may be employed either alone or in combination with physical entanglement as mentioned above.

The binder is desirably of such a type as to turn into a non-fibrous carbonized product through the carbonization treatment for the production of the heat-insulating, carbon fiber felting material according to the present invention. Specific examples of the binder include those including at least one member selected from among phenolic resins, furan resins, amino resins, tar, and pitch.

The use of the binder such as the above-mentioned specific resin or tar permits the felting material according to the present invention to take a considerably complicated shape because mat-like or felty carbon fiber materials may be not only simply piled up but also further formed into such a complicated shape through interfiber adhesion with the binder such as the resin or tar at the middle stage of entanglement.

##### (C) Binderless Entanglement

According to the present invention, without use of the above-mentioned binder, a pitch fiber prior to carbonization (precursor fiber) can be self-bonded at the time of carbonization to keep the morphology thereof felty. In this case, physical entanglement such as needle punching may be combined with such self-bonding.

In the foregoing pitch fiber self-bonding method, the infusibilization treatment is effected under such weak conditions as not to bring about complete infusibilization of the fiber while keeping the fiber morphology in a stable state.

In order to enhance the self-bonding properties of the pitch fiber, a precursor fiber which is readily infusibilized may be blended with a precursor fiber which is not readily infusibilized, provided that at least one of the precursor fibers is a pitch fiber. According to this method, the morphology-retaining properties of the fiber easy of infusibilization can be fully utilized, while at the same time adhesion of the fiber not easy of infusibilization can be utilized.

Examples of the precursor fiber readily infusibilized include those derived from polyacrylonitrile, cellulose, a phenolic resin, or optically anisotropic pitch. Examples of the precursor fiber not easy of infusibilization include those derived from optically isotropic pitch, polyvinyl alcohol, or aramids.

The precursor fiber not readily infusibilized sometimes cannot keep the morphology at the time of carbonization. This problem can be solved when use is made of a blended yarn produced by bicomponent spinning of the precursor fiber not readily infusibilized and the precursor fiber readily infusibilized.

#### HEAT-INSULATING CARBON FIBER FELTING MATERIAL

The carbon fiber felting material of the present invention, which is characterized by interfiber entanglement as described hereinbefore, has a bulk density of 0.01 to 0.5 g/cm<sup>3</sup>, preferably 0.05 to 0.5 g/cm<sup>3</sup>, and a thermal conductivity of at most 1.0 kcal/m·hr·°C., preferably at most 0.7 kcal/m hr °C., as measured in the thickness-wise direction of the felting material at 2,200° C.

The bulk density of the felting material of the present invention is 0.01 to 0.5 g/cm<sup>3</sup>, preferably 0.05 to 0.5 g/cm<sup>3</sup>, because the porosity of the felting material is desired to be increased as use as possible by making much of any gas included therein in order to enhance the heat insulating effect thereof.

The heat insulating effect of the felting material is enhanced as the bulk density of the felting material is increased, in so far as the carbon fiber in the felting material is not oriented in a continuous state in the direction of the Z axis.

When the bulk density is lower than 0.01 g/cm<sup>3</sup>, the radiation-scattering effect of the felting material may be lowered to increase the thermal conductivity thereof. When the bulk density is so high as to exceed 0.5 g/cm<sup>3</sup>, the thermal conductivity is increased as well to lower the heat insulating effect of the felting material.

The bulk density of the felting material can be adjusted to a predetermined level by controlling the needle punching density during entanglement, the pressure applied thereto during carbonization, and/or equivalent processes known in the art.

In the case where a binder to be converted into a non-fibrous carbonized product is in a state of being applied on the felting material of the present invention, the carbon fiber content of the felting material is preferably in the range of about 60 to 95 wt. %, more preferably about 70 to about 90 wt. %. Conversely speaking, the content of the binder matrix convertible into the non-fibrous carbonized product in the felting material is preferably in the range of about 5 to about 40 wt. %, more preferably about 10 to about 30 wt. %.

In other words, it is not preferable from the viewpoint of the heat insulating properties of the felting material that either the carbon fiber or the binder matrix be continuous in the thickness-wise direction of the felting material (in the direction of Z axis in which heat insulation is desired). In this respect, it is believed that either the carbon fiber or the binder matrix is preferably oriented only in parallel with the X-Y plane of the felting material.

In general, the binder matrix is used to keep the desired shape of felting material resistant to processing and the like. Point-wise interfiber adhesion is generally preferable, while the amount of the binder matrix itself is preferably as small as possible. In order to keep the desired shape of felting material, however, it is necessary to use some amount of the binder matrix. In this sense, the binder matrix content of the felting material is usually about 5 to 40 wt. %.

The term "carbon fiber content" as well as "binder matrix content" used herein is intended to indicate a value calculated based on the yield of carbon or graphite formed by individual heat treatment of a fiber as well as a binder.

The method of measuring the thermal conductivity of carbon fiber felting material as specified in the present invention is in accordance with JIS A 1412 "Procedure of Measuring Thermal Conductivity of Heat Insulating Material" except for use of a radiation pyrometer instead of a thermocouple as specified in JIS for the measurement of temperature, the use of which is difficult in this case.

The carbon fiber felting material of the present invention has a thermal conductivity of at most 1.0 kcal/m·hr·°C., preferably at most 0.7 kcal/m·hr·°C. as measured in the thickness-wise direction of the felting material at a temperature of 2,200° C.

As described hereinabove, the carbon fiber felting material of the present invention is of technological significance in that it is (a) constituted of a thin carbon fiber having an average filament diameter of, for example, 1 to 9  $\mu$ m and (b) subjected to such interfiber entanglement as to have a high bulk density of 0.01 to 0.5 g/cm<sup>3</sup>, preferably 0.05 to 0.5 g/cm<sup>3</sup>, with the result that it (c) can exhibit a very high heat insulating effect as demonstrated above in terms of thermal conductivity, and especially an excellent heat insulation performance against radiant heat transfer, and that it (d) is useful as a heat-insulating material at high temperatures since the carbon fiber is a material that can be used stably in an inert atmosphere up to about 2,800° C.

#### PRODUCTION OF CARBON FIBER FELTING MATERIAL

In brief, the carbon fiber felting material of the present invention is preferably produced through the step (1) of spinning a starting pitch material by a melt blow method and collecting the spun fiber into the form of a sheet, the step (2) of subjecting the fiber sheet to infusibilization and subsequent slight carbonization treatments, and the step (3) of piling up a desired number of the resultant carbon fiber sheets and subsequently entangling the carbon fiber sheets with each other, followed by carbonization of the resultant mat if desired.

##### Entanglement

Specifically, entanglement may be effected through [a] a physical entanglement treatment such as needle punching at a density of 2 to 100 punches/cm<sup>2</sup> and/or

[b] a chemical entanglement treatment comprising impregnation of the carbon fiber mats with at least one substance selected from among phenolic resins, furan resins, amino resins, tar and pitch, subsequent curing of a resin if used, and carbonization of the impregnating substance into a non-fibrous carbonized product, or [c] a chemical entanglement treatment comprising infusibilization of pitch fiber sheets obtained in the step (1) under such conditions as to bring about interfiber self-bonding thereof at the time of carbonization, and piling-up and subsequent carbonization of a desired number of infusibilized pitch fiber sheets.

The process for producing a carbon fiber felting material according to the present invention will now be described in detail.

#### Step (1)

##### [1] Production of Pitch Fiber

The spinning step of producing a pitch fiber (precursor fiber) may employ an arbitrary spinning method such as a centrifugal spinning method, a spun-bonding method, and a melt blow method, which is especially preferable because thin filaments can be relatively easily produced thereby.

As the filaments are thinner, the curvature radius of the filaments are naturally smaller to show a tendency to have a higher capability of radiation scattering on the surfaces thereof, which is believed to greatly contribute to heat insulation against radiant heat transfer.

Furthermore, thinner filaments are known to contribute to heat insulation against convectional heat transfer. In view of the foregoing, a carbon fiber produced through melt blow spinning is believed to be excellent in heat insulating properties in the high-temperature range.

Among pitch fibers employable in the present invention, a pitch fiber produced through melt blow spinning is especially excellent as a material for forming a heat-insulating felting material.

The reason is that such a pitch fiber is generally not linear but curled or crimped. Non-linear parts of the fiber provide room for permitting fiber movement during needle punching to lower the probability of fiber breakage and increase the proportion of fibers inclined relative to the surfaces of the resulting sheet at the sites of interfiber entanglement. This results in a reduction of through-fiber conductive heat transfer, leading to an advantage of unhindered heat-insulating effect.

The use of a mesophase pitch type carbon fiber in particular provides a low-moisture-absorption carbon fiber felting material.

Specifically, in the case of melt blow spinning, spinning may usually be done through spinning orifices provided in a nozzle or a slit, which ejects a gas at a high speed, under spinning conditions involving a spinneret temperature of 290° to 360° C., a gas temperature of 310° to 380° C., and a gas ejection rate of 100 to 340 m/sec.

##### [2] Collection of Spun Fiber into the Form of Sheet

In the process of the present invention, the spun fiber is preferably collected into the form of a sheet in a step directly associated with the spinning step to produce a mat-like material. This is advantageous in that no fibrous material is contained in the final product because the opening and/or carding step liable to give damage to a fiber having a small elongation can be dispensed

with unlike in conventional processes for producing a non-woven fabric.

The fibrous material presents a problem of contaminating the surroundings or clogging the filter(s) of an air conditioner during the service of a heat insulating material because of its high mobility.

The method of collecting a spun fiber into the form of a sheet in a step directly associated with the spinning step is advantageous in that sheets can generally be produced in low cost.

#### [3] Production of Mat-like Material

In the process of the present invention, if necessary, the pitch fiber sheet obtained by collecting the spun fiber into the form of 1 sheet in the step (a) may be continuously cross-lapped to form a mat-like material (sheet laminate) uniform thereacross in unit weight.

#### Step (d)

In the process of the present invention, the infusibilization and slight carbonization treatments may be arbitrarily done according to customary methods.

##### [1] Infusibilization Treatment

For example, the infusibilization treatment may be done through a heat treatment effected in an atmosphere of an oxidizing gas such as air, oxygen or NO<sub>x</sub> at a heat-up rate of 0.2° to 13° C./min, preferably 2° to 10° C./min, up to a temperature of 200° to 400° C.

##### [2] Carbonization Treatment

Where carbonization is followed by a physical entanglement treatment such as needle punching, a slight carbonization treatment is preferably effected. For example, carbonization is effected in an inert gas such as nitrogen gas at a heat-up rate of 5° to 100° C./min up to a temperature of 300° to 1,500° C., preferably 500° to 1,000° C., according to a customary method.

#### Step (3)

##### [1] Physical Entanglement Treatment

A necessary number of the resulting infusibilized and carbonized fiber sheets are piled up in accordance with the purpose and use thereof and subjected to a physical entanglement treatment such as needle punching, which usually has to be done at a density of 2 to 100 punches/cm<sup>2</sup>.

Alternatively, the gas turbulence method, the columnar liquid stream penetration method, or the like may of course be employed.

According to any of these methods which can be carried out with a superior shape stability of felting material, however, a carbon fiber is sometimes oriented in the thickness-wise direction of a felting material being formed during the course of entanglement to lower the heat insulating effect of the felting material because the thermal conductivity of the felting material is higher in the direction of the carbon fiber. Thus, care should be taken to minimize such orientation of the carbon fiber.

In the case of needle punching, when the needle punch density was lower than 2 punches/cm<sup>2</sup>, the resulting carbon fiber felting material is weakened in strength to unfavorably present a problem of poor handleability. When the needle punch density exceeds 100 punches/cm<sup>2</sup>, the content of carbon fibers oriented in a direction perpendicular to the surface of a felting mate-

rial being formed is increased to raise the thermal conductivity related to conductive heat transfer. This results in an unfavorable decrease in the heat insulating effect of the felting material. In addition, attendant fiber breakage unfavorably lowers the strength of the felting material.

[2] Chemical Entanglement Treatment

a Impregnation with Binder

It is preferable that the mat-like material already subjected to the physical entanglement treatment such as needle punching (of course, the mat-like material may not be subjected to any physical entanglement treatment) be impregnated with a binder matrix capable of turning into a non-fibrous carbonized product upon carbonization, which is at least one substance selected from the group consisting of phenolic resins, furan resins, amino resins, tar and pitch, to effect such point-wise interfiber adhesion as to be able to keep the mat-like material in a desired morphology.

In this case, the amount of the impregnating binder matrix may be minimum if only it is at least sufficient to retain the shape of felting material. The binder matrix content of the felting material is preferably in the range of about 5 to 40 wt. %.

b Curing of Binder

The impregnating binder matrix is subsequently cured, for example, by heating according to a customary method.

c Carbonization of Binder and the Like

Finally, the mat-like material thus treated is carbonized according to a customary method. For example, this can be done through a heat treatment in an inert gas such as nitrogen gas at a temperature of 900° to 2,000° C. for a given period of time.

Besides the foregoing kind of felting material simply comprising laminated sheets, the felting material of the present invention is able to have a considerably complicated shape because such a shape may be provided by interfiber adhesion with a resin or tar in the intermediate step (d).

(3) Binderless Entanglement Treatment

Without the use of a binder and without any physical entanglement treatment such as needle punching, entanglement may be effected through such a weak infusibilization treatment of a pitch fiber prior to carbonization as to effect incomplete infusibilization though the shape of the fiber is stabilized during the course of carbonization.

Suitable infusibilization conditions are preferably determined using the degree of oxygen inclusion of the infusibilized fiber as a yardstick. The term "degree of oxygen inclusion" used herein is intended to mean the percentage of the oxygen content of the infusibilized fiber relative to the oxygen content of the completely infusibilized fiber, the degree of oxygen inclusion of which is naturally 100%. Incomplete infusibilization is desirably effected up to a degree of oxygen inclusion of 30 to 95%, preferably 40 to 75%.

Specifically, the heat-up rate during the course of infusibilization may be set slow. For example, the temperature may be elevated to a predetermined infusibilization temperature of about 250° to 300° C. at a heat-up rate of about 1° to 3° C./min, followed by termination of heating before complete infusibilization. In this case,

the resulting infusibilized fiber is in such an incompletely infusibilized state as to have self-bonding properties at the time of carbonization. The timing of termination of heating can be easily found by checking the oxygen content of the fiber. The oxygen content can be easily examined through elemental analysis of the infusibilized fiber to determine the degree of oxygen inclusion.

Heat transfer in a high temperature range wherein radiant heat transfer is dominant is considerably dissimilar from heat transfer in a low temperature range wherein convective heat transfer and conductive heat transfer are predominant.

The carbon fiber felting material of the present invention is so superior in the capability of absorbing as well as scattering a radiation contributory to radiant heat transfer that it is highly effective in heat insulation against radiant heat transfer.

A reason for the great heat-insulating effect against radiant heat transfer which the felting material of the present invention can exhibit is thin filaments used therein which have a small surface curvature radius. A smaller surface curvature radius provides the felting material with a larger capability of radiation scattering, which is believed to greatly contribute to heat insulation against radiant heat transfer.

The reason why a precursor pitch fiber produced by the melt blow method is especially excellent among various starting materials usable to produce the carbon fiber felting material of the present invention is general non-linearity of the fiber including many curls and crimps. Non-linear parts of the fiber provide such room for fiber movement as to reduce the chances of fiber breakage and increase the proportion of fibers inclined relative to the surface of the mat-like material at the sites of interfiber entanglement. This reduces through-fiber conductive heat transfer to provide an advantage of not spoiling the heat-insulating effect of the resulting felting material, which is otherwise in substantial proportion to the degree of entanglement.

BEST MODES FOR CARRYING OUT THE INVENTION

The following Examples will now specifically illustrate the present invention, but should not be construed as limiting the scope of the invention.

Physical Entanglement

EXAMPLE 1

Petroleum pitch having a softening point of 284° C. and a mesophase content of 100% was used as a starting material to form a pitch fiber according to the melt blow method. The fiber was collected on a net conveyor to form a sheet.

The pitch fiber sheet was infusibilized by heating in air at a heat-up rate of 2.4° C./min to 300° C., and then slightly carbonized by heating in nitrogen gas at a heat-up rate of 5° C./min to 615° C.

The average filament diameter of the resulting slightly carbonized fiber was 6.5  $\mu$ m, while the unit weight of the resulting sheet formed thereof was 28 g/m<sup>2</sup>.

12 pieces of the sheet were piled up and subjected to needle punching. Felty materials produced at respective punch densities as listed in Table 1 were carbonized at a maximum temperature of 2,000° C.

The bulk density of the mat before punching was varied by the pressure applied thereto during slight

carbonization to adjust the bulk density of the felting material after carbonization to  $0.1 \pm 0.01 \text{ g/cm}^3$ .

Additionally stated, a felty material produced at a punch density of 1.8 punches/cm<sup>2</sup> was not so good in coherence to show a tendency to exfoliate relatively easily into a number of sheets in the course of handling.

The moisture absorptions of all the felting materials produced in the foregoing manner were about 0.08%. The thermal conductivities of the felting materials as measured at 2,200° C. with a thermal conductivity measurement device for heat insulating materials (Model ITC25-VR11 manufactured by Ishikawajima-Harima Heavy Industries Co., Ltd.) are listed together with punch densities in Table 1.

TABLE 1

| Run No.                            | 1    | 2    | 3    | 4    | 5    |
|------------------------------------|------|------|------|------|------|
| Punch Density* <sup>1</sup>        | 1.8  | 7    | 35   | 95   | 100  |
| Thermal Conductivity* <sup>2</sup> | 0.52 | 0.60 | 0.68 | 0.77 | 1.12 |

\*<sup>1</sup> punches/cm<sup>2</sup>

\*<sup>2</sup> kcal/m · hr · °C.

Runs Nos. 1 to 4 are of Example, while Run No. 5 is of Comparative Example.

### EXAMPLE 2

The infusibilized sheets prepared in the same manner as in Example 1 were slightly carbonized under varied pressures applied thereto to obtain sheets having various bulk densities.

12 pieces of each kind of sheets having the same bulk density were subjected to needle punching at a density of 7 punches/cm<sup>2</sup> to produce a felting material.

The bulk densities of felting materials produced in the foregoing manner are listed in Table 2.

The thermal conductivities of the felting materials, measured at 2,200° C. in the same manner as in Example 1, are listed in Table 2.

TABLE 2

| Run Nos.                           | 1     | 2    | 3    | 4    | 5    |
|------------------------------------|-------|------|------|------|------|
| Bulk Density* <sup>1</sup>         | 0.008 | 0.02 | 0.08 | 0.45 | 0.59 |
| Thermal Conductivity* <sup>2</sup> | 1.23  | 0.86 | 0.60 | 0.85 | 1.30 |

\*<sup>1</sup> g/cm<sup>3</sup>

\*<sup>2</sup> kcal/m · hr · °C.

Runs Nos. 2 to 4 are of Example, while Runs Nos. 1 and 5 are of Comparative Example.

### EXAMPLE 3

Isotropic coal pitch having a softening point of 238° C. as the starting material was spun and collected into the form of a sheet in the same manner as in Example 1, followed by infusibilization and slight carbonization thereof in the same manner as in Example 1 (average filament diameter after slight carbonization: 7 μm). The resulting sheets were piled up and subjected to needle punching in the same manner as in Example 1 to form a felting material.

The thermal conductivity of the felting material, measured at 2,200° C. in the same manner as in Example 1, was 0.92 kcal/m · hr · °C. The moisture absorption of 60 the felting material was about 5 wt. %.

### EXAMPLE 4

The same mesophase petroleum pitch as in Example 1 was spun and collected into the form of a sheet in substantially the same manner as in Example 1 except that the amount per orifice of pitch spun was varied to form fibers having different filament diameters. In substan-

tially the same manner as in Example 1, each kind of pitch fiber sheet formed of fibers having the same average filament diameter was then infusibilized, slightly carbonized in a weakly compressed state, piled up, and subjected to needle punching at a density of 7 punches/cm<sup>2</sup> to form a felting material.

The average filament diameters of the fibers after slight carbonization thereof were listed in Table 3. The bulk densities of the felting materials were  $0.1 \pm 0.01 \text{ g/cm}^3$ . The thermal conductivities of the felting materials, measured at 2,200° C. in the same manner as in Example 1, are listed in Table 3. The moisture absorptions of the felting materials were 0.03 to 1.8 wt. %.

TABLE 3

| Run No.                                 | 1    | 2    | 3    | 4    | 5    |
|-----------------------------------------|------|------|------|------|------|
| Average Filament Diameter* <sup>1</sup> | 1.2  | 3.6  | 8.7  | 11.0 | 16.0 |
| Thermal Conductivity* <sup>2</sup>      | 0.18 | 0.44 | 0.78 | 1.13 | 3.25 |

\*<sup>1</sup> μm

\*<sup>2</sup> kcal/m · hr · °C.

Runs Nos. 1 to 3 are of Example, while Runs Nos. 4 and 5 are of Comparative Example.

### Entanglement with Binder

### EXAMPLE 5

Petroleum pitch having a softening point of 284° C. and a mesophase content of 100% was used as the starting material to spin a pitch fiber according to the melt blow method. The pitch fiber was collected on a net conveyor to form a pitch fiber sheet having a unit weight of 30 g/m<sup>2</sup>.

The sheet thus obtained continuously was piled up with a horizontal crosslapper to obtain a laminated sheet having a uniform unit weight of 600 g/m<sup>2</sup>.

This laminated pitch fiber sheet was infusibilized by heating in air at a heat-up rate of 5° C./min up to 300° C., and subsequently slightly carbonized by heating in nitrogen gas at a heat-up rate of 5° C./min up to 615° C., followed by needle punching at a density of 13 punches/cm<sup>2</sup>.

Two pieces of the resulting mats having a bulk density of 0.11 g/cm<sup>3</sup> were piled up and impregnated with a resol phenolic resin ("Plyophen" manufactured by Dainippon Ink & Chemicals, Inc.) in such an amount as to provide a fiber content of 90 wt. %. The impregnated mats were heated at 165° C. to cure the resin. The resulting mat was carbonized at a maximum temperature of 2,000° C. to produce a felting material having a bulk density of 0.15 g/cm<sup>3</sup>.

The average filament diameter of the fiber in the felting material was 6.5 μm. The thermal conductivity of the felting material, measured at 2,200° C. with a thermal conductivity measurement device for heat insulating materials (Model ITC25-VR11 manufactured by Ishikawajima-Harima Heavy Industries Co., Ltd.), was 0.26 kcal/m · hr · °C.

### EXAMPLE 6

The infusibilized sheets prepared in the same manner as in Example 5 were slightly carbonized under varied pressures applied thereto to obtain mats having various bulk densities, followed by needle punching at a density of 7 punches/cm<sup>2</sup>.

Two pieces of each kind of the needle-punched mat were piled up and impregnated with the same resol

phenolic resin as used in Example 5 in such an amount as to provide a fiber content of 90 wt. %. The impregnated mats were heated at 165° C. to cure the resin, and totally carbonized by heating up to 2,000° C. to produce a felting material (heat-insulating material).

The thermal conductivities of the resulting felting materials, measured in the same manner as in Example 5, are listed together with the bulk densities thereof in Table 4.

The average filament diameter of the fiber after carbonization was 6.5  $\mu\text{m}$ .

TABLE 4

| Run No.                            | 1    | 2    | 3    | 4    | 5    |
|------------------------------------|------|------|------|------|------|
| Bulk Density* <sup>1</sup>         | 0.02 | 0.09 | 0.2  | 0.41 | 0.57 |
| Thermal Conductivity* <sup>2</sup> | 0.91 | 0.25 | 0.31 | 0.65 | 1.08 |

\*<sup>1</sup>g/cm<sup>3</sup>

\*<sup>2</sup>kcal/m · hr · °C.

Runs Nos. 1 to 4 are of Example, while Run No. 5 is Comparative Example.

## EXAMPLE 7

Isotropic coal pitch having a softening point of 238° C. as the starting material was spun and collected into the form of a sheet in the same manner as in Example 5, followed by infusibilization and slight carbonization thereof in the same manner as in Example 5. The resulting mats were piled up and subjected to needle punching in the same manner as in Example 5 to form a felty material.

Two pieces of the resulting felty materials were piled up and impregnated with the same resol phenolic resin as used in Example 5 in such an amount as to provide a fiber content of 90 wt. %. The impregnated felty materials were heated to cure the resin and carbonized in the same manner as in Example 5. The thermal conductivity of the resulting felting material, measured in the same manner as in Example 5, was 0.60 kcal/m·hr·°C.

The average filament diameter of the fiber after carbonization was 7  $\mu\text{m}$ .

## EXAMPLE 8

The same mesophase petroleum pitch as in Example 5 was spun and collected into the form of a sheet in substantially the same manner as in Example 5 except that the amount per orifice of pitch spun was varied to form fibers having different filament diameters. The resulting fiber sheets were infusibilized and slightly carbonized in substantially the same manner as in Example 5. Two pieces of each type of the resulting sheet were piled up and subjected to needle punching at a density of 7 punches/cm<sup>2</sup> to form a felty material. The felty material was then impregnated with the same resol phenolic resin as used in Example 5, heated to cure the resin, and carbonized in the same manner as in Example 5 to produce a felting material having a bulk density of 0.1 g/cm<sup>3</sup>.

The average filament diameters and thermal conductivities of the felting materials (heat-insulating materials) thus produced, measured in the same manner as in Example 5, are shown in Table 5.

TABLE 5

| Run No.                                 | 1   | 2   | 3   | 4    | 5    |
|-----------------------------------------|-----|-----|-----|------|------|
| Average Filament Diameter* <sup>1</sup> | 1.2 | 3.6 | 8.7 | 11.0 | 16.0 |

TABLE 5-continued

| Run No.                            | 1    | 2    | 3    | 4    | 5    |
|------------------------------------|------|------|------|------|------|
| Thermal Conductivity* <sup>2</sup> | 0.17 | 0.23 | 0.42 | 1.06 | 1.25 |

\*<sup>1</sup> $\mu\text{m}$

\*<sup>2</sup>kcal/m · hr · °C.

Runs Nos. 1 to 3 are of Example, while Runs Nos. 4 and 5 are a Comparative Examples.

## 10 Binderless Entanglement

## EXAMPLE 9

Petroleum pitch having a softening point of 284° C. and a mesophase content of 100% was used as the starting material to spin a pitch fiber according to the melt blow method. The fiber was collected on a net conveyor to form a pitch fiber sheet, which was then heated in air at a heat-up rate of 1° C./min up to 250° C. to be infusibilized.

The oxygen content of the resulting infusibilized fiber at this stage was determined to be 70% of the oxygen content of the completely infusibilized fiber.

15 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 894

a sheet in substantially the same manner as in Example 9. The resulting pitch fiber sheet was heated in air at a heat-up rate of 1.2° C./min up to 240° C. to be so infusiblized as to be still self-bondable. The infusiblized sheets were piled up and slightly carbonized to produce a felting material (average filament diameter after slight carbonization: 7  $\mu\text{m}$ ).

The thermal conductivity of the felting material, measured in the same manner as in Example 9, was 0.92 kcal/m·hr·°C. The moisture absorption of the felting material was about 5.5 wt. %.

#### EXAMPLE 12

The same mesophase petroleum pitch as used in Example 9 was spun and collected into the form of a sheet in substantially the same manner as in Example 9 except that the amount per orifice of pitch spun was varied to form fibers having different average filament diameters. Each kind of resulting fiber sheet formed of fibers having the same average filament diameter were heated in air at a heat-up rate of 1.3° C./min up to 245° C. to be so infusiblized as to be still self-bondable, piled up, and slightly carbonized in a weakly compressed state to produce a felting material.

The average filament diameters of the slightly carbonized fibers are listed in Table 7. The bulk densities of the felting materials were  $0.1 \pm 0.01 \text{ g/cm}^3$ .

The thermal conductivities of the felting materials, measured in the same manner as in Example 9, are listed in Table 7. The moisture absorptions of the felting materials were 0.05 to 1.9 wt. %.

TABLE 7

| Run No.                                 | 1    | 2    | 3    | 4    | 5    |
|-----------------------------------------|------|------|------|------|------|
| Average Filament Diameter* <sup>1</sup> | 1.3  | 3.4  | 8.6  | 11.2 | 16.4 |
| Thermal Conductivity* <sup>2</sup>      | 0.19 | 0.42 | 0.76 | 1.09 | 2.75 |

\*<sup>1</sup> $\mu\text{m}$

\*<sup>2</sup>kcal/m · hr · °C.

Runs Nos. 1 to 3 are of Example, while Runs Nos. 4 and 5 are of Comparative Example.

The carbon fiber felting material of the present invention is very stable in an inert atmosphere and exhibits excellent heat resistance and morphological stability within the temperature range of 500° to 2,800° C. as well as excellent heat insulating properties against radiant heat transfer.

The carbon fiber felting material of the present invention is so excellent in heat insulating properties in the

50

55

60

high-temperature range that it can be used for heat insulation of high temperature furnaces which are used in fusion of glass, firing of pottery, smelting of metals, sintering of ceramics, or heat treatment of carbonaceous materials.

The carbon fiber felting material of the present invention is so excellent in stability against radiation that it can be used as a heat-insulating material with excellent performance in nuclear furnaces and nuclear power generating installations.

The heat-insulating, carbon fiber felting material of a mesophase pitch type in particular according to the present invention is so low in moisture absorption that the problems or troubles attributed to evaporation of water at the time of heat-up of a heat-insulating material and high-temperature water vapor can be avoided to favorably prevent deterioration of the carbon fiber felting material itself and to advantageously shorten the operation time of, for example, a furnace due to the ability of the heat-insulating material to allow for heat-up thereof in a short time without any troubles.

What is claimed is:

1. A melt-blown pitch type carbon fiber felting material excellent in heat insulating properties in a high-temperature range, which is substantially in the form of a felt formed of a pitch type carbon fiber through interfiber entanglement and having a bulk density of 0.01 to 0.5  $\text{g/cm}^3$ , a thermal conductivity of at most 1.0 kcal/m·hr·°C. in the thickness-wise direction thereof at a temperature of 2,200° C., and an average filament diameter of 1 to 9  $\mu\text{m}$ .

2. A carbon fiber felting material as claimed in claim 1, wherein said carbon fiber is of a mesophase pitch type, and which has a moisture absorption of at most 2 wt. % as measured in an atmosphere having a temperature of 200° C. and a relative humidity of 65%.

3. A process for producing a carbon fiber felting material excellent in heat insulating properties as claimed in claim 1: comprising the step (1) of spinning a starting pitch material by a melt blow method and collecting the spun fiber into the form of a sheet, the step (2) of subjecting the fiber sheet to infusiblization and subsequent slight carbonization treatments, and the step (3) of piling up a desired number of the resultant carbon fiber sheets and subsequently entangling said carbon fiber sheets with each other, followed by carbonization of the resultant mat if desired.

\* \* \* \* \*

65